

## UNITED STATES PATENT OFFICE

2,263,366

## SUPPRESSING COKING ON SURFACES

Edward B. Peck, Elizabeth, and Peter J. Gaylor,  
Union, N. J., assignors to Standard Oil Develop-  
ment Company, a corporation of Delaware

No Drawing. Application June 24, 1939,  
Serial No. 281,052

2 Claims. (Cl. 196—47)

This invention deals with a method for inhibiting or retarding the formation of coke and tarry matter upon heated surfaces in contact with organic materials.

Coking and carbonization difficulties have been encountered in industrial equipment such as cracking coils, vacuum distillation towers, combustion chambers of automotive engines, heat transfer equipment and the like. An object of the present invention is to retard or eliminate such coking or deposition of tarry materials which hinder and interfere with the operation of the equipment employed for commercial uses.

The present invention involves the coating of the surface in contact with the organic substance with a layer comprising zinc oxide. A large number of elements and compounds have been tried, but it has been found that only zinc oxide exhibits a strong enough inhibiting effect against coking to justify its commercial use. Although it is possible to coat surfaces with zinc oxide by the use of paints, varnishes or lacquers containing at least 25% or preferably 50% or more zinc oxide, there are three processes which are recommended for obtaining satisfactorily adhering zinc oxide films especially upon metallic surfaces. The first method involves the electro deposition of a thin zinc layer upon the cleaned metallic surface followed by conversion of the zinc film to zinc oxide by anodic oxidation, chemical oxidation, such as with dichromates, or heating in presence of air or oxygen for a limited length of time. The second method involves the treatment of the metal surface with zinc vapors in presence of reducing gases for such a period of time as to allow the zinc to penetrate into the metal to such an extent as to form a bonded surface, after which oxidation of the zinc surface is carried out as set forth above. The third method consists in galvanizing the metallic surface or spraying the surface with the molten metal in a reducing atmosphere followed by the oxidation procedure. With these processes, it is

possible to obtain a homogeneous adherent coating of zinc oxide which will withstand vibration and mechanical handling without loss of the protective coating.

5 Such coatings may be applied to the metallic or other surfaces which have a tendency to coke or collect tarry deposits. Ferrous and nickel surfaces are especially noted for their coke-collecting tendencies.

10 Zinc oxide also tends to suppress the cracking of organic compounds, and in this respect it is valuable where cracking is to be avoided. Hence, it may be employed as a coating or ingredient for a catalyst employed in thermal reactions such as cracking, dehydrogenation, reforming, isomerization, polymerization, etc. Zinc compounds readily convertible into zinc oxide on oxidation may also be employed dissolved or dispersed in lubricants and fuels so as to prevent deposition of coke or similar materials in combustion engines. It is preferable, however, that the surface to be made substantially free of carbon be coated with zinc oxide to obtain the best results.

We claim:

1. A method of thermally cracking hydrocarbons to produce gasoline in a reaction container made of metal containing iron and nickel which have coke forming characteristics, which comprises coating the internal surface of said metal reaction container with a homogeneous adherent protective coating of zinc oxide and then heating hydrocarbons in said reaction container having an internal zinc oxide coating to a cracking temperature for a sufficient time to effect the desired extent of cracking.

2. A method according to claim 1 wherein the zinc is deposited as a thin film of metal on the internal surface of said reaction container and then is oxidized to form an adherent layer of zinc oxide before said container is used for cracking hydrocarbons.

EDWARD B. PECK.  
PETER J. GAYLOR.